# EUROPEAN PATENT SPECIFICATION

(11) **EP 3 951 049 B1**
(45) Date of publication and mention of the grant of the patent: **10.01.2024**
(21) Application number: 21166623.5
(22) Date of filing: 01.04.2021
(51) Int. Cl.: D21H 11/14, D21H 19/58, D21H 21/34, D21H 27/10, D21H 27/30

(54) **HIGH-PERFORMANCE ENVIRONMENT-FRIENDLY KRAFT LINER BOARD, AND PREPARATION METHOD THEREOF**
HOCHLEISTUNGSFÄHIGE, UMWELTFREUNDLICHE KRAFTLINER-PLATTE UND HERSTELLUNGSVERFAHREN DAFÜR
PANNEAU DE DOUBLURE KRAFT ÉCOLOGIQUE HAUTE PERFORMANCE ET SON PROCÉDÉ DE PRÉPARATION

(30) Priority: 06.08.2020 CN 202010587201
(43) Date of publication of application: 09.02.2022
(73) Proprietor: Zhejiang Rongsheng Environmental Protection Paper Co., Ltd., Zhejiang (CN)
(72) Inventor: FENG, Ronghua, Pinghu Economic Development Zone, Zhejiang (CN); FENG, Shengyu, Pinghu Economic Development Zone, Zhejiang (CN); CHEN, Jiandong, Pinghu Economic Development Zone, Zhejiang (CN); LU, Xiaojun, Pinghu Economic Development Zone, Zhejiang (CN); HU, Rongxia, Pinghu Economic Development Zone, Zhejiang (CN); WU, Xiaomin, Pinghu Economic Development Zone, Zhejiang (CN)
(74) Representative: Chung, Hoi Kan

(56) References cited:
- CN-A- 108 385 435
- CN-A- 109 853 282
- CN-B- 108 385 426
- CN-B- 108 505 372
- US-A1- 2010 279 113

## Description

### TECHNICAL FIELD

The present invention relates to the manufacturing and processing technical field of carton boards, in particular to a high-performance environment-friendly kraft liner board, and a preparation method thereof.

### BACKGROUND

Carton boards are the most important raw materials for wrapping cartons. With the improvement of people's living standards and social progress, many high-grade cartons for commodity wrapping need to consume a large number of high-performance carton boards. With the continuous development of China's paper industry, the shortage of fiber raw materials has become a bottleneck issue that restricts sustainable development of the paper industry. Thus, waste paper which is widely applied in carton boards manufacturing enterprises also limits the improvement of product performance.

The technical problems need to be solved by the present invention are described as follow:

Currently, kraft liner boards for various wrapping cartons are generally made of waste paper, and without utilizing flame retardant treatment in most cases. However, some high-grade wrapping cartons or special products, such as export products, a small number of high-grade consumer products, flammable and explosive products, military products, require flame retardant wrapping and transportation in particular. Moreover, electric commercial cartons, whether they are ordinary cartons or cartons for wrapping color TVs, refrigerators and other high-grade electrical appliances, the kraft liner boards used among them are generally without flame retardant treatment, it is a hidden danger, fires happen occasionally during transportation or storage of wrapping cartons. With the development of society and the improvement of people's living requirements, it is an inevitable requirement to treat kraft liner boards with flame retardants for wrapping cartons. In the prior art, some wrapping carton products adopt the method of adding plenty of flame retardants in the pulp to get the flame retardant performance, but the added amount is large, the effect is limited, the cost is high, and the physical strength of the products is affected.

For example, one of the prior arts i.e., Chinese Patent Number: CN108505372B discloses a kind of method for producing low gram weight and high strength degree craft paper using domestic waste paper. Also, another prior art i.e., Chinese Patent Number: CN109853282A discloses a kind of fire-retardant kraft liner board prepared using fire-retardant secondary stock. However, said prior arts fail to disclose production of a paper/kraft liner board with a flame retardant layer that is effective in terms of flame retardant properties and cost, and also that does not impact the strength of the paper/ kraft liner board while adding the flame retardant properties.

Solving the surface performance, water resistance and strength problems of high-performance carton boards.

Conventionally, kraft liner boards are used to wrap higher-grade products, so they have higher requirements on their quality performance, especially in the process of box making, such as stretching and folding, which requires good folding endurance, tensile strength, and ring crush compression strength. After being made into cartons, good bursting strength and water resistance are required during wrapping and transportation. In order to improve the wrapping effect, the surface requires exquisite printing, so kraft liner boards also require good surface smoothing performance. The prior art mainly adopts surface sizing method to improve the ring crush compression strength and surface water resistance of products, which has many defects: surface sizing can mainly improve the surface strength and partial ring crush compression resistance of the products, but have limited effect on improving the overall physical strength of the products, such as tensile strength, bursting strength and folding endurance, so the physical properties of the kraft liner boards mainly produced by waste paper are restricted. Therefore, a large number of reinforcing agents require to be added in the production process to solve the problems, and the loss is large and the cost is high. Moreover, the usage of surface sizing has a certain effect on improving the surface water resistance and lowering the Cobb value of the product, but it has limited effect on improving the overall water resistance of the kraft liner boards. Furthermore, the usage of surface sizing can improve the surface smoothness of the products to a certain extent, but it is difficult to achieve the effect of high-quality wrapping and printing products.

Based on above reasons, the present invention is provided.

### SUMMARY

Aiming at above problems or defects in the prior art, objects of the present invention are to provide a high-performance environment-friendly kraft liner board, and a preparation method thereof. The invention is set out in the appended set of claims.

In order to accomplish the first object, the present invention adopts technical solutions as follows.

A high-performance environment-friendly kraft liner board, comprising a bottom layer, a top layer and a coating layer, which are arranged successively in an order from bottom to top; wherein: the bottom layer is made of a bottom layer pulp composed of a modified wood powdery pulp and a short fiber pulp; the top layer is made of a top layer pulp composed of a long fiber pulp and a short fiber pulp; the coating layer is formed through coating a flame retardant styrene-acrylic latex on the top layer; the long fiber pulp and the short fiber pulp are formed through pulping old domestic corrugated boxes; the flame retardant styrene-acrylic latex consists of modified composite flame retardants, a functional modified styrene-acrylic latex and water.

Further, in the above technical solution, a basis weight of the high-performance environment-friendly kraft liner board is 100-120 g/m², a ring pressure index is 6.7-7.6 mN·m²/g, a frontal water absorption is 30-31 g/m², and a limit oxygen index is 30-33%, a smoothness is 15-16 seconds, a bursting index is 2.4-2.6 kPa·m²/g, and a folding endurance is 15-20 times.

Further, in the above technical solution, a weight percentage concentration of the flame retardant styrene-acrylic latex is 2.0-5.0%.

Further, in the above technical solution, a weight ratio of the modified composite flame retardants to the functional modified styrene-acrylic latex is 1:2.5-3.0.

Further, in the above technical solution, the modified composite flame retardants are prepared through modifying composite flame retardants with a modifier; wherein: the modifier is a silane coupling agent; more preferably, the silane coupling agent is N-( β-aminoethyl)-r-aminopropyltrimethoxysilane.

Further, in the above technical solution, a weight ratio of the modifier to the composite flame retardants is (0.002-0.01):1.

Further, in the above technical solution, the composite flame retardants contain two or more flame retardant elements. For example, the composite flame retardants may be a combination of any two or more of ammonium polyphosphate, polyphosphoester, melamine polyphosphate, zinc borate, aluminum phosphate, aluminum hydroxide, etc., and a ratio of each flame retardant element is not specifically limited.

Preferably, in the above technical solution, the composite flame retardants consist of two or more flame retardant elements of equal weight.

Preferably, in the above technical solution, the zinc borate are ultra-fine powders with a particle size of 0.02-0.04 um.

Preferably, in the above technical solution, the aluminum hydroxide are ultra-fine powders with a particle size of 0.03-0.05 um.

Further, in the above technical solution, a preparation method of the modified composite flame retardants is as follows: mixing the composite flame retardants with the modifier, and stirring evenly.

Further, in the above technical solution, the functional modified styrene-acrylic latex is prepared through steps of:

according to a proportion, adding dicyclopentenyl methacrylate, water, sodium dodecyl sulfate and nonylphenol polyoxyethylene ether into a reactor 1, stirring evenly; adding trimethylene carbonate, after stirring evenly, successively adding acrylic acid, hydroxyethyl acrylate, butyl acrylate and styrene into reaction system, stirring at a constant speed until mixing well; thereafter, heating the reaction system to 70-90°C, adding sodium bicarbonate and a initiator, under stirring condition, a reaction is carried out at constant temperature for 2-4 hours, upon completion of the reaction, cooling to a room temperature, filtering, adjusting a pH value of an obtained product to neutral, and obtaining the functional modified styrene-acrylic latex.

Further, in the above technical solution, a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate and the initiator is 1:40-50:0.2-0.3:0.3-0.4:1-1.3:0.2-0.5:4-6: 25-35:25-35:0.2-0.4:0.4-0.6.

Preferably, in the above technical solution, the initiator is a persulfate salt, and specifically can be any one of ammonium persulfate, sodium persulfate or potassium persulfate.

Preferably, in the above technical solution, a pH regulator adopts ammonia water.

Specifically, in the above technical solution, a structural formula of the dicyclopentenyl methacrylate is shown in following formula 1:

More preferably, in the above technical solution, the dicyclopentenyl methacrylate is prepared through steps of:

according to a proportion, successively adding methacrylic acid, trifluoromethanesulfonic acid and hydroquinone to a reactor 2, after stirring and mixing well, heating to 78-82°C, adding dicyclopentadiene to the reactor 2, mixing well, then heating reaction system to 85-90°C, a reaction is carried out at constant temperature for 3-4 hours, upon completion of the reaction, cooling to a room temperature, adding sodium hydroxide (NaOH) into an obtained product, stirring for 1-2 hours, finally washing an obtained mixture, filtering, distilling, and obtaining the dicyclopentenyl methacrylate.

Most preferably, in the above technical solution, an agitator speed is 100-500 r/min.

Most preferably, in the above technical solution, a weight ratio of the methacrylic acid, the trifluoromethanesulfonic acid, the hydroquinone, the dicyclopentadiene and the NaOH is 0.8-1.2:0.002-0.004:0.00006-0.0001:1.5-2.0:0.0015-0.002.

Further, in the above technical solution, a weight percentage concentration of the long fiber pulp is 3.5-4.5%, a weight percentage concentration of the short fiber pulp is 4-5%, and a weight percentage concentration of the modified wood powdery pulp is 3-5%.

Further, in the above technical solution, in the bottom layer pulp, a weight ratio of the modified wood powdery pulp to the short fiber pulp is 5-10:95-90.

Further, in the above technical solution, the modified wood powdery pulp is prepared through modifying wood powders with a swelling agent, and the swelling agent is a mixed alkali; a modification method is as follows: after processing the wood powders with a refiner, successively adding the mixed alkali and water, stirring evenly, then heating an obtained mixture to 70-90°C, and a swelling treatment is carried out at constant temperature for 60-90 minutes to form the modified wood powdery pulp.

preferably, in the above technical solution, the mixed alkali consists of sodium hydroxide and sodium carbonate; wherein: amounts of each raw material are calculated by weight, wood powders: sodium hydroxide: sodium carbonate=1: 0.01-0.03:0.01-0.03.

preferably, in the above technical solution, the water used for the swelling agent modifying wood powders adopts dryer condensed water in a double-stacked paper machine, which is used for preparing products of the present invention.

Further, in the above technical solution, in the top layer pulp, a weight ratio of the long fiber pulp to the short fiber pulp is 80-90:20-10.

Further, in the above technical solution, a weight ratio of the top layer pulp to the bottom layer pulp is 40-50:60-50.

Further, in the above technical solution, a ratio of total weight of absolute dry fibers contained in the bottom layer pulp and the top layer pulp to a weight of the coating layer is 1:0.005-0.015.

A second object of the present invention is to provide a preparation method for the above high-performance environment-friendly kraft liner board, comprising steps of:
(1) pulping steps
   (i)preparation of a long fiber pulp and a short fiber pulp
      deflaking old domestic corrugated boxes with a hydrapulper, separating dregs at a high consistency, then coarse screening for first level three stages, screen sizing to a long fiber coarse pulp and a short fiber coarse pulp; separating the long fiber coarse pulp for first level three stages, removing dregs; successively fine screening obtained fibers for first level three stages, thicking with a multi-disc thickener, refining with a conical refiner, and finally diluting with water to obtain the long fiber pulp, storing in a machine chest for use; successively fine screening the short fiber coarse pulp for first level two stages and refining with the conical refiner, finally diluting with water to obtain the short fiber pulp, storing in a pulp chest for use;
   (ii)preparation of a modified wood powdery pulp
      processing wood powders with a refiner, successively adding a mixed alkali and water, stirring evenly, heating an obtained mixture to 70-90°C, and a swelling treatment is carried out at constant temperature for 60-90 minutes, so as to soften fibers appropriately and form the modified wood powdery pulp with a weight percentage concentration of 3-5%;
(2) papermaking steps
   according to a proportion, mixing the modified wood powdery pulp and the short fiber pulp obtained through the step (1) uniformly to form a bottom layer pulp, mixing the long fiber pulp and the short fiber pulp uniformly to form a top layer pulp; then flowing the bottom layer pulp and the top layer pulp on wire respectively, adding retention and drainage aids to the approach flow system, double-folding, laminating, pressing, drying, coating, calendering and reeling to obtain the high-performance environment-friendly kraft liner board.

Further, in the above technical solution, in the step(i), a first-stage pressure screen of the fine screening for first level three stages adopts a micro-slot width pressure screen to remove binders, and a screen slot width is 0.08-0.12 mm.

Further, in the above technical solution, in the step(i), a weight ratio of absolute dry long fibers in the long fiber coarse pulp obtained by screen sizing to absolute dry short fibers in the short fiber coarse pulp is 30-40:70-60.

Further, in the above technical solution, in the step(i), the long fiber pulp adopts conical refiners in series to refine the pulp, and adopts a long fiber viscous beating technology, and a beating degree is 28-30 °SR.

Further, in the above technical solution, in the step(i), a weight percentage concentration of the long fiber pulp is 3.5-4.5%, and a weight percentage concentration of the short fiber pulp is 4-5%.

Further, in the above technical solution, the water in the step (i) and step (ii) both adopts dryer condensed water in a double-stacked paper machine.

Further, in the above technical solution, the retention and drainage aids in the step (2) consist of two components: cationic polyacrylamide and silica sol, wherein: a weight ratio of absolute dry fibers, cationic polyacrylamide, and silica sol is 1:0.001-0.002:0.001-0.002; the absolute dry fibers refer to total amounts of absolute dry fibers contained in the bottom layer pulp and the top layer pulp.

Further, in the above technical solution, the coating in the step (2) adopts the metering roller coating technology, specifically, by a metering roller coating method, coating the flame retardant styrene-acrylic latex on the top layer of the kraft liner board obtained through double-folding, laminating, pressing and drying, so as to form a coating layer.

Compared with the prior art, the beneficial effects of the present invention are described as follows:
(1) The present invention adopts composite flame retardant latex metering roller coating method to add the flame retardants, which is no loss and low cost, moreover, the addition of the flame retardants has no adverse effects on the strength of the paper.
(2)The present invention adopts acrylic acid, hydroxyethyl acrylate, butyl acrylate, styrene as reactive monomers, adopts trimethylene carbonate, dicyclopentenyl methacrylate as functional monomers, and adopts a emulsion polymerization method to prepare the functional modified styrene-acrylic latex, then combines it with the flame retardants to prepare the flame retardant styrene-acrylic latex; thereafter, through coating method to prepare the high-performance environment-friendly kraft liner board. The functional modified styrene-acrylic latex of the present invention can replace or partially replace the reinforcing agent, sizing agent and other auxiliary agents added in the pulp during production of the kraft liner board, so that the product has good overall physical strength and water resistance. Moreover, the present invention adopts the metering roller coating method, which improves the smoothness of the surface of the kraft liner board product, greatly improves the printing effect, and raises the level of the product.
(3) The functional modified styrene-acrylic latex prepared by the present invention is combined with the composite flame retardants containing multiple flame retardant elements to obtain the flame retardant latex, which can fully exert the synergistic flame retardant effect of the multiple flame retardants.
(4) The preparation process of the present invention is advanced, pollution-free and low production cost, moreover, the prepared kraft liner board has good physical strength, water resistance and flame retardancy. Because the kraft box preparation product of the present invention is produced from all waste paper, the process is environment-friendly and the functional modified styrene-acrylic latex is a water-soluble latex without organic solvents, which improves environmental protection.

### BRIEF DESCRIPTION OF DRAWINGS

FIG.1 is a preparation process flow chart of the high-performance environment-friendly kraft liner board according to the present invention.

### DETAILED DESCRIPTION OF THE EMBODIMENTS

The present invention is further illustrated in detail with examples. The examples are implemented on the premise of the technology according to the present invention. Now detailed implementation and specific operation process are given to illustrate the creativity of the present invention, but the protection scope of the present invention is not limited to the following examples.

Based on the information contained in this application, it is easy for those skilled in the art to make various changes to the precise description of the present invention without departing from the spirit and scope of the appended claims. It should be understood that the scope of the present invention is not limited to the defined processes, properties, or components, because these examples and other descriptions are merely intended to illustrate specific aspects of the present invention. In fact, various changes that can be made to the examples of the present invention by those skilled in the art or related fields are all encompassed in the scope of the appended claims.

In order to better understand the present invention without limiting the scope of the present invention, all numbers expressing dosages, percentages, and other numerical values used in this application should be understood as modified by the word "about" in all cases. Therefore, unless otherwise specified, the numerical parameters listed in the specification and the appended claims are approximate values, which may be changed according to the desired properties that are attempted to be obtained. Each numerical parameter should at least be regarded as obtained based on the reported significant figures and through conventional rounding methods.

The materials and reagents used in the following examples can be obtained from commercial sources unless otherwise specified.

A high-performance environment-friendly kraft liner board is disclosed that comprises a bottom layer, a top layer and a coating layer, which are arranged successively in an order from bottom to top. The bottom layer is made of a bottom layer pulp composed of a modified wood powdery pulp and a short fiber pulp. The top layer is made of a top layer pulp composed of a long fiber pulp and a short fiber pulp. The coating layer is formed through coating a flame retardant styrene-acrylic latex on the top layer. The long fiber pulp and the short fiber pulp are formed through pulping old domestic corrugated boxes. The flame retardant styrene-acrylic latex consists of modified composite flame retardants, a functional modified styrene-acrylic latex and water.

The composite flame retardants are a combination of any two or more of ammonium polyphosphate, polyphosphoester, melamine polyphosphate, zinc borate, and aluminum phosphate; a weight ratio of the modified composite flame retardants to the functional modified styrene-acrylic latex is 1:2.5-3.0. The modified composite flame retardants are prepared through modifying composite flame retardants with a silane coupling agent.

The functional modified styrene-acrylic latex is prepared through steps of: adding according to a proportion, dicyclopentenyl methacrylate, water, sodium dodecyl sulfate and nonylphenol polyoxyethylene ether into a reactor 1 and stirring evenly. Then adding trimethylene carbonate, and after stirring evenly, successively adding acrylic acid, hydroxyethyl acrylate, butyl acrylate and styrene into reaction system, while stirring at a constant speed until they are mixed well. Further, the reaction system is heated to 70-90°C, and sodium bicarbonate and an initiator are added and stirred. Under stirring condition, a reaction is carried out at constant temperature for 2-4 hours, and upon completion of the reaction, the mixture is cooled to a room temperature. Thereafter, filtering is done and a pH value of an obtained product is adjusted to neutral, and obtaining the functional modified styrene-acrylic latex.

The proportion includes a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate and the initiator is 1:40-50:0.2-0.3:0.3-0.4:1-1.3:0.2-0.5:4-6: 25-35:25-35:0.2-0.4:0.4-0.6.

### Example 1

In this example, the method for preparing a high-performance environment -friendly kraft liner board, comprising following steps of:
(1) preparing for a flame retardant styrene-acrylic latex
   (a) preparing for a dicyclopentenyl methacrylate
      according to a proportion, successively adding methacrylic acid, trifluoromethanesulfonic acid and hydroquinone to a reactor 2 equipped with an agitator, controlling an agitator speed of the agitator to 210 r/min, after stirring and mixing well, heating to 80°C; then adding dicyclopentadiene, controlling a reaction temperature of reaction system to 85°C, a reaction is carried out at constant temperature for 3.5 hours, upon completion of the reaction, cooling to a room temperature, adding NaOH and stirring for 1.5 hours, washing an obtained mixture, filtering, distilling, and obtaining the dicyclopentenyl methacrylate; wherein: the weight ratio of the methacrylic acid, the trifluoromethanesulfonic acid, the hydroquinone, the dicyclopentadiene, and the NaOH is 1:0.0028:0.000095:1.72:0.0018;
   (b)preparing for a functional modified styrene-acrylic latex
      the functional modified styrene-acrylic latex is prepared through following method, particularly comprising steps of:
      according to a proportion, adding dicyclopentenyl methacrylate obtained in the step(a), water, sodium dodecyl sulfate and nonylphenol polyoxyethylene ether into a reactor 1, stirring evenly; adding trimethylene carbonate, after stirring evenly, successively adding acrylic acid, hydroxyethyl acrylate, butyl acrylate and styrene into reaction system, stirring at a constant speed until mixing well; thereafter, heating the reaction system to 80°C, adding sodium bicarbonate and ammonium persulfate, under stirring condition, a reaction is carried out at constant temperature for 4 hours, upon completion of the reaction, cooling to a room temperature, filtering, adjusting a pH value of an obtained product to neutral with aqueous ammonia solution, and obtaining the functional modified styrene-acrylic latex;
      wherein: a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate and the ammonium persulfate is 1:40:0.2:0.3:1:0.2:4:25:25:0.2:0.4;
   (c)preparing for the flame retardant styrene-acrylic latex
      mixing modifier N-(β-aminoethyl)-r-aminopropyltrimethoxysilane and composite flame retardants at a weight ratio of 0.002:1, stirring evenly, and obtaining modified composite flame retardants; then mixing the modified composite flame retardants and the functional modified styrene-acrylic latex prepared in the step (a) uniformly at a weight ratio of 1:2.5, diluting with water, and obtaining the flame retardant styrene-acrylic latex with a weight percentage concentration of 2.0%; the water adopts dryer condensed water;
      wherein: the composite flame retardants consist of zinc borate and aluminum hydroxide with a weight ratio of 1:1; the zinc borate and aluminum hydroxide are both ultra-fine powders, and a particle size of the zinc borate is 0.02-0.04 um; a particle size of the aluminum hydroxide is 0.03-0.05 um;
(2) pulping steps
   (i) preparation of a long fiber pulp and a short fiber pulp
      deflaking old domestic corrugated boxes with a hydrapulper, separating dregs at a high consistency, then coarse screening for first level three stages, screen sizing to a long fiber coarse pulp and a short fiber coarse pulp; separating the long fiber coarse pulp for first level three stages, removing dregs; successively fine screening obtained fibers for first level three stages, thicking with a multi-disc thickener, refining with a conical refiner, and finally diluting with water to obtain the long fiber pulp, storing in a machine chest for use; successively fine screening the short fiber coarse pulp for first level two stages and refining with the conical refiner, finally diluting with water to obtain the short fiber pulp, storing in a pulp chest for use; the water used in this step all adopts dryer condensed water in a double-stacked paper machine;
      wherein: a first-stage pressure screen of the fine screening for first level three stages adopts a micro-slot width pressure screen to remove binders, and a screen slot width is 0.08-0.12 mm;
      a weight ratio of absolute dry long fibers in the long fiber coarse pulp obtained by screen sizing to absolute dry short fibers in the short fiber coarse pulp is 40:60;
      the long fiber pulp adopts conical refiners in series to refine the pulp, and adopts a long fiber viscous beating technology, and a beating degree is 28 °SR;
      a weight percentage concentration of the long fiber pulp is 3.5%, and a weight percentage concentration of the short fiber pulp is 5%;
   (ii)preparation of a modified wood powdery pulp
      processing wood powders with a refiner, successively adding a mixed alkali and water, stirring evenly, heating an obtained mixture to 70°C, and a swelling treatment is carried out at constant temperature for 60 minutes, so as to soften fibers appropriately and form the modified wood powdery pulp with a weight percentage concentration of 3%;
      wherein: the mixed alkali consists of sodium hydroxide and sodium carbonate; the water adopts dryer condensed water in a double-stacked paper machine;
      in the step (ii), amounts of each raw material are calculated by weight, wood powders: sodium hydroxide: sodium carbonate=1:0.01:0.01;
(3) papermaking steps
   mixing the modified wood powdery pulp and the short fiber pulp obtained in the step (2) uniformly at a weight ratio of 10:90 to form a bottom layer pulp; mixing the long fiber pulp and the short fiber pulp obtained in the step (3) uniformly at a weight ratio of 80:20 to form a top layer pulp; then flowing the bottom layer pulp and the top layer pulp on wire respectively, adding retention and drainage aids to the approach flow system, double-folding, laminating, pressing, drying, coating, calendering and reeling to obtain the high-performance environment-friendly kraft liner board;
   wherein: a weight ratio of the top layer pulp to the bottom layer pulp is 40:60;
   the retention and drainage aids consist of two components: cationic polyacrylamide and silica sol, a weight ratio of absolute dry fibers, cationic polyacrylamide, and silica sol is 1:0.001:0.001; the absolute dry fibers refer to total amounts of absolute dry fibers contained in the bottom layer pulp and the top layer pulp;
   the coating process adopts the metering roller coating technology, specifically, by a metering roller coating method, coating the flame retardant styrene-acrylic latex on the top layer of the kraft liner board obtained through double-folding, laminating, pressing and drying, so as to form a coating layer;
   a ratio of the total weight of the absolute dry fibers contained in the bottom layer pulp and the top layer pulp to a weight of the coating layer is 1 :0.005.

### Example 2

In this example, the preparation method of a high-performance environment -friendly kraft liner board, comprising following steps of:
(1) preparing for a flame retardant styrene-acrylic latex
   (a) preparing for a dicyclopentenyl methacrylate
      according to a proportion, successively adding methacrylic acid, trifluoromethanesulfonic acid and hydroquinone to a reactor 2 equipped with an agitator, after stirring and mixing well under 100 r/min condition, heating to 78°C; then adding dicyclopentadiene into the reactor 2, mixing well, heating reaction system to 90°C, a reaction is carried out at constant temperature for 3 hours, upon completion of the reaction, cooling to a room temperature, adding NaOH into an obtained product, stirring for 1h, finally washing an obtained mixture, filtering, distilling, and obtaining the dicyclopentenyl methacrylate; wherein: the weight ratio of the methacrylic acid, the trifluoromethanesulfonic acid, the hydroquinone, the dicyclopentadiene, and the NaOH is 0.8:0.002:0.00006:1.5:0.0015;
   (b)preparing for a functional modified styrene-acrylic latex
      the functional modified styrene-acrylic latex is prepared through following method, particularly comprising steps of:
      according to a proportion, adding dicyclopentenyl methacrylate obtained in the step(a), water, sodium dodecyl sulfate and nonylphenol polyoxyethylene ether into a reactor 1, stirring evenly; adding trimethylene carbonate, after stirring evenly, successively adding acrylic acid, hydroxyethyl acrylate, butyl acrylate and styrene into reaction system, stirring at a constant speed until mixing well; thereafter, heating the reaction system to 70°C, adding sodium bicarbonate and ammonium persulfate, under stirring condition, a reaction is carried out at constant temperature for 3 hours, upon completion of the reaction, cooling to a room temperature, filtering, adjusting a pH value of an obtained product to neutral with aqueous ammonia solution, and obtaining the functional modified styrene-acrylic latex;
      wherein: a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate and the ammonium persulfate is 1:45:0.25:0.35:1.2:0.3:5:30:30:0.3:0.5;
   (c)preparing for the flame retardant styrene-acrylic latex
      mixing modifier N-(β-aminoethyl)-r-aminopropyltrimethoxysilane and composite flame retardants at a weight ratio of 0.005:1, stirring evenly, and obtaining modified composite flame retardants; then mixing the modified composite flame retardants and the functional modified styrene-acrylic latex prepared in the step (a) uniformly at a weight ratio of 1:2.8, diluting with water, and obtaining the flame retardant styrene-acrylic latex with a weight percentage concentration of 3.5%; the water adopts dryer condensed water in a double-stacked paper machine;
      wherein: the composite flame retardants consist of ammonium polyphosphate, polyphosphoester and zinc borate with a weight ratio of 1:1:1; the zinc borate are ultra-fine powders, and a particle size of the zinc borate is 0.02-0.04 um;
(2) pulping steps
   (i) preparation of a long fiber pulp and a short fiber pulp
      deflaking old domestic corrugated boxes with a hydrapulper, separating dregs at a high consistency, then coarse screening for first level three stages, screen sizing to a long fiber coarse pulp and a short fiber coarse pulp; separating the long fiber coarse pulp for first level three stages, removing dregs; successively fine screening obtained fibers for first level three stages, thicking with a multi-disc thickener, refining with a conical refiner, and finally diluting with water to obtain the long fiber pulp, storing in a machine chest for use; successively fine screening the short fiber coarse pulp for first level two stages and refining with the conical refiner, finally diluting with water to obtain the short fiber pulp, storing in a pulp chest for use; the water used in this step all adopts dryer condensed water in a double-stacked paper machine;
      wherein: a first-stage pressure screen of the fine screening for first level three stages adopts a micro-slot width pressure screen to remove binders, and a screen slot width is 0.08-0.12 mm;
      a weight ratio of absolute dry long fibers in the long fiber coarse pulp obtained by screen sizing to absolute dry short fibers in the short fiber coarse pulp is 30:70;
      the long fiber pulp adopts conical refiners in series to refine the pulp, and adopts a long fiber viscous beating technology, and a beating degree is 30 °SR;
      a weight percentage concentration of the long fiber pulp is 4.0%, and a weight percentage concentration of the short fiber pulp is 4.5%;
   (ii)preparation of a modified wood powdery pulp
      processing wood powders with a refiner, successively adding a mixed alkali and water, stirring evenly, heating an obtained mixture to 90°C, and a swelling treatment is carried out at constant temperature for 70 minutes, so as to soften fibers appropriately and form the modified wood powdery pulp with a weight percentage concentration of 4%;
      wherein: the mixed alkali consists of sodium hydroxide and sodium carbonate; the water adopts dryer condensed water in a double-stacked paper machine;
      in the step (ii), amounts of each raw material are calculated by weight, wood powders: sodium hydroxide: sodium carbonate=1:0.02:0.02;
(3) papermaking steps
   mixing the modified wood powdery pulp and the short fiber pulp obtained in the step (2) uniformly at a weight ratio of 5:95 to form a bottom layer pulp; mixing the long fiber pulp and the short fiber pulp obtained in the step (3) uniformly at a weight ratio of 90:10 to form a top layer pulp; then flowing the bottom layer pulp and the top layer pulp on wire respectively, adding retention and drainage aids to the approach flow system, double-folding, laminating, pressing, drying, coating, calendering and reeling to obtain the high-performance environment-friendly kraft liner board;
   wherein: a weight ratio of the top layer pulp to the bottom layer pulp is 50:50;
   the retention and drainage aids consist of two components: cationic polyacrylamide and silica sol, wherein: a weight ratio of absolute dry fibers, cationic polyacrylamide, and silica sol is 1:0.0015:0.0015; the absolute dry fibers refer to total amounts of absolute dry fibers contained in the bottom layer pulp and the top layer pulp;
   the coating process adopts the metering roller coating technology, specifically, by a metering roller coating method, coating the flame retardant styrene-acrylic latex on the top layer of the kraft liner board obtained through double-folding, laminating, pressing and drying, so as to form a coating layer;
   a ratio of the total weight of the absolute dry fibers contained in the bottom layer pulp and the top layer pulp to a weight of the coating layer is 1:0.01.

### Example 3

In this example, the preparation method of a high-performance environment -friendly kraft liner board, comprising following steps of:
(1) prepareing for a flame retardant styrene-acrylic latex
   (a) prepareing for a dicyclopentenyl methacrylate
      according to a proportion, successively adding methacrylic acid, trifluoromethanesulfonic acid and hydroquinone to a reactor 2 equipped with an agitator, after stirring and mixing well under 500 r/min condition, heating to 82°C; then adding dicyclopentadiene into the reactor 2, mixing well, heating reaction system to 85°C, a reaction is carried out at constant temperature for 4 hours, upon completion of the reaction, cooling to a room temperature, adding NaOH into an obtained product, stirring for 2 hours, finally washing an obtained mixture, filtering, distilling, and obtaining the dicyclopentenyl methacrylate; wherein: the weight ratio of the methacrylic acid, the trifluoromethanesulfonic acid, the hydroquinone, the dicyclopentadiene, and the NaOH is 1.2:0.004:0.0001: 2.0:0.002;
   (b)preparing for a functional modified styrene-acrylic latex
      the functional modified styrene-acrylic latex is prepared through following method, particularly comprising steps of:
      according to a proportion, adding dicyclopentenyl methacrylate obtained in the step(a), water, sodium dodecyl sulfate and nonylphenol polyoxyethylene ether into a reactor 1, stirring evenly; adding trimethylene carbonate, after stirring evenly, successively adding acrylic acid, hydroxyethyl acrylate, butyl acrylate and styrene into reaction system, stirring at a constant speed until mixing well; thereafter, heating the reaction system to 85°C, adding sodium bicarbonate and ammonium persulfate, under stirring condition, a reaction is carried out at constant temperature for 2 hours, upon completion of the reaction, cooling to a room temperature, filtering, adjusting a pH value of an obtained product to neutral with aqueous ammonia solution, and obtaining the functional modified styrene-acrylic latex;
      wherein: a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate and the ammonium persulfate is 1:50:0.3:0.4:1.3:0.5:6:35:35: 0.4:0.6;
   (c)preparing for the flame retardant styrene-acrylic latex
      mixing modifier N-(β-aminoethyl)-r-aminopropyltrimethoxysilane and composite flame retardants at a weight ratio of 0.01:1, stirring evenly, and obtaining modified composite flame retardants; then mixing the modified composite flame retardants and the functional modified styrene-acrylic latex prepared in the step (a) uniformly at a weight ratio of 1:3.0, diluting with water, and obtaining the flame retardant styrene-acrylic latex with a weight percentage concentration of 5%; the water adopts dryer condensed water in a double-stacked paper machine;
      wherein: the composite flame retardants consist of ammonium polyphosphate, polyphosphoester and melamine polyphosphate with a weight ratio of 1:1:1;
(2) pulping steps
   (i) preparation of a long fiber pulp and a short fiber pulp
      deflaking old domestic corrugated boxes with a hydrapulper, separating dregs at a high consistency, then coarse screening for first level three stages, screen sizing to a long fiber coarse pulp and a short fiber coarse pulp; separating the long fiber coarse pulp for first level three stages, removing dregs; successively fine screening obtained fibers for first level three stages, thicking with a multi-disc thickener, refining with a conical refiner, and finally diluting with water to obtain the long fiber pulp, storing in a machine chest for use; successively fine screening the short fiber coarse pulp for first level two stages and refining with the conical refiner, finally diluting with water to obtain the short fiber pulp, storing in a pulp chest for use; the water used in this step all adopts dryer condensed water in a double-stacked paper machine;
      wherein: a first-stage pressure screen of the fine screening for first level three stages adopts a micro-slot width pressure screen to remove binders, and a screen slot width is 0.08-0.12 mm;
      a weight ratio of absolute dry long fibers in the long fiber coarse pulp obtained by screen sizing to absolute dry short fibers in the short fiber coarse pulp is 35:65;
      the long fiber pulp adopts conical refiners in series to refine the pulp, and adopts a long fiber viscous beating technology, and a beating degree is 30 °SR;
      a weight percentage concentration of the long fiber pulp is 4.5%, and a weight percentage concentration of the short fiber pulp is 5%;
   (ii)preparation of a modified wood powdery pulp
      processing wood powders with a refiner, successively adding a mixed alkali and water, stirring evenly, heating an obtained mixture to 80°C, and a swelling treatment is carried out at constant temperature for 90 minutes, so as to soften fibers appropriately and form the modified wood powdery pulp with a weight percentage concentration of 5%;
      wherein: the mixed alkali consists of sodium hydroxide and sodium carbonate; the water adopts dryer condensed water in a double-stacked paper machine;
      in the step (ii), amounts of each raw material are calculated by weight, wood powders: sodium hydroxide: sodium carbonate=1:0.03:0.03;
(3) papermaking steps
   mixing the modified wood powdery pulp and the short fiber pulp obtained in the step (2) uniformly at a weight ratio of 8:92 to form a bottom layer pulp; mixing the long fiber pulp and the short fiber pulp obtained in the step (3) uniformly at a weight ratio of 85:15 to form a top layer pulp; then flowing the bottom layer pulp and the top layer pulp on wire respectively, adding retention and drainage aids to the approach flow system, double-folding, laminating, pressing, drying, coating, calendering and reeling to obtain the high-performance environment-friendly kraft liner board;
   wherein: a weight ratio of the top layer pulp to the bottom layer pulp is 45:55;
   the retention and drainage aids consist of two components: cationic polyacrylamide and silica sol, wherein: a weight ratio of absolute dry fibers, cationic polyacrylamide, and silica sol is 1:0.002:0.002; the absolute dry fibers refer to total amounts of absolute dry fibers contained in the bottom layer pulp and the top layer pulp;
   the coating process adopts the metering roller coating technology, specifically, by a metering roller coating method, coating the flame retardant styrene-acrylic latex on the top layer of the kraft liner board obtained through double-folding, laminating, pressing and drying, so as to form a coating layer;
   a ratio of the total weight of the absolute dry fibers contained in the bottom layer pulp and the top layer pulp to a weight of the coating layer is 1:0.015.

The main performance indexes of the high-performance environment-friendly kraft liner board prepared in the examples 1 to 3 are tested. The ring pressure index is tested according to an GB/T2679.8-2016 "Paperboard-Determination of ring crush compression strength"; the frontal water absorption is tested according to an GB/T1540-2002 "Paper and board-Determination of water absorption"; the flame retardancy is tested according to an oxygen index meter ASTM D2863 standard; smoothness is tested according to an GB/T456-2002 "Paper and board-Determination of smoothness" (Bekk method); bursting index is tested according to an GB/T1539-2007 "Paperboard-Determination of bursting strength"; Folding endurance is tested according to an GB/T2679.5-2002 "Paper and board-Determination of folding endurance ". The test results are shown in Table 1.

**Table 1 The main performance index test results of the high-performance environment-friendly kraft liner board prepared in Examples 1-3.**

| Technical indexes | Example 1 | Example 2 | Example 3 |
|---|---|---|---|
| a basis weight (g/m²) | 100 | 120 | 110 |
| a ring pressure index (mN·m²/g) | 6.7 | 7.6 | 7.2 |
| a frontal water absorption (g/m²) | 30 | 31 | 30.6 |
| flame retardancy | 30 | 33 | 32.4 |
| (a limit oxygen index %) | | | |
| a smoothness (seconds) | 15 | 16 | 16 |
| a bursting index (kPa·m²/g ) | 2.4 | 2.6 | 2.55 |
| a folding endurance (times) | 15 | 20 | 20 |

## Claims

1. A high-performance environment-friendly kraft liner board, comprising a bottom layer, a top layer and a coating layer, which are arranged successively in an order from bottom to top; wherein: the bottom layer is made of a bottom layer pulp composed of a modified wood powdery pulp and a short fiber pulp; the top layer is made of a top layer pulp composed of a long fiber pulp and a short fiber pulp; the coating layer is formed through coating a flame retardant styrene-acrylic latex on the top layer; the long fiber pulp and the short fiber pulp are formed through pulping old domestic corrugated boxes; the flame retardant styrene-acrylic latex consists of modified composite flame retardants, a functional modified styrene-acrylic latex and water; the composite flame retardants are a combination of any two or more of ammonium polyphosphate, polyphosphoester, melamine polyphosphate, zinc borate, aluminium hydroxide, and aluminum phosphate; the modified composite flame retardants are prepared through modifying composite flame retardants with a silane coupling agent;
a weight ratio of the modified composite flame retardants to the functional modified styrene-acrylic latex is 1:2.5-3.0; the modified composite flame retardants are prepared through modifying composite flame retardants with a silane coupling agent;
the functional modified styrene-acrylic latex is prepared through steps of:
according to a proportion, adding dicyclopentenyl methacrylate, water, sodium dodecyl sulfate and nonylphenol polyoxyethylene ether into a reactor 1, stirring evenly; adding trimethylene carbonate, after stirring evenly, successively adding acrylic acid, hydroxyethyl acrylate, butyl acrylate and styrene into reaction system, stirring at a constant speed until mixing well; thereafter, heating the reaction system to 70-90°C, adding sodium bicarbonate and a initiator, under stirring condition, a reaction is carried out at constant temperature for 2-4 hours, upon completion of the reaction, cooling to a room temperature, filtering, adjusting a pH value of an obtained product to neutral, and obtaining the functional modified styrene-acrylic latex, the proportion includes a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate and the initiator is 1:40-50:0.2-0.3:0.3-0.4:1-1.3:0.2-0.5:4-6: 25-35:25-35:0.2-0.4:0.4-0.6.

2. The high-performance environment-friendly kraft liner board, as recited in claim 1, wherein: a basis weight of the high-performance environment-friendly kraft liner board is 100-120 g/m², a ring pressure index is 6.7-7.6 mN·m²/g, a frontal water absorption is 30-31 g/m², and a limit oxygen index is 30-33%, a smoothness is 15-16 seconds, a bursting index is 2.4-2.6 kPa·m²/g, and a folding endurance is 15-20 times.

3. The high-performance environment-friendly kraft liner board, as recited in claim 1, wherein: the dicyclopentenyl methacrylate is prepared through steps of:
according to a proportion, successively adding methacrylic acid, trifluoromethanesulfonic acid and hydroquinone to a reactor 2, after stirring and mixing well, heating to 78-82°C, adding dicyclopentadiene to the reactor 2, mixing well, then heating reaction system to 85-90°C, a reaction is carried out at constant temperature for 3-4 hours, upon completion of the reaction, cooling to a room temperature, adding sodium hydroxide into an obtained product, stirring for 1-2 hours, finally washing an obtained mixture, filtering, distilling, and obtaining the dicyclopentenyl methacrylate; and the trifluoromethanesulfonic acid, the hydroquinone, the dicyclopentadiene and the NaOH is 0.8-1.2:0.002-0.004:0.00006-0.0001:1.5-2.0:0.0015-0.002.

4. The high-performance environment-friendly kraft liner board, as recited in claim 1, wherein: the proportion includes a weight ratio of the dicyclopentenyl methacrylate, the water, the sodium dodecyl sulfate, the nonylphenol polyoxyethylene ether, the trimethylene carbonate, the acrylic acid, the hydroxyethyl acrylate, the butyl acrylate, the styrene, the sodium bicarbonate, and the initiator is 1:40-50:0.2-0.3:0.3-0.4:1-1.3:0.2-0.5:4-6:25-35:25-35:0.2-0.4:0.4-0.6.

5. The high-performance environment-friendly kraft liner board, as recited in claim 1, the modified wood powdery pulp is prepared through modifying wood powders with a swelling agent, and the swelling agent is a mixed alkali; a modification method is as follows: after processing the wood powders with a refiner, successively adding the mixed alkali and water, stirring evenly, then heating an obtained mixture to 70-90°C, and a swelling treatment is carried out at constant temperature for 60-90 minutes to form the modified wood powdery pulp; wherein: the mixed alkali consists of sodium hydroxide and sodium carbonate.

6. A preparation method for the high-performance environment-friendly kraft liner board as recited in claim 1, wherein: comprising steps of:
(1) pulping steps
(i) preparation of a long fiber pulp and a short fiber pulp
- deflaking old domestic corrugated boxes with a hydrapulper, separating dregs at a high consistency, then coarse screening for first level three stages, screen sizing to a long fiber coarse pulp and a short fiber coarse pulp;
- separating the long fiber coarse pulp for first level three stages, removing dregs;
- successively fine screening obtained fibers for first level three stages, thicking with a multi-disc thickener, refining with a conical refiner, and finally diluting with water to obtain the long fiber pulp, storing in a machine chest for use;
- successively fine screening the short fiber coarse pulp for first level two stages and refining with the conical refiner, finally diluting with water to obtain the short fiber pulp, storing in a pulp chest for use;
(ii) preparation of a modified wood powdery pulp
- processing wood powders with a refiner, successively adding a mixed alkali and water, stirring evenly, heating an obtained mixture to 70-90°C, and a swelling treatment is carried out at constant temperature for 60-90 minutes, so as to soften fibers appropriately and form the modified wood powdery pulp with a weight percentage concentration of 3-5%;
(2) papermaking steps
- according to a proportion, mixing the modified wood powdery pulp and the short fiber pulp obtained through the step (1) uniformly to form a bottom layer pulp,
- mixing the long fiber pulp and the short fiber pulp uniformly to form a top layer pulp;
- then flowing the bottom layer pulp and the top layer pulp on wire respectively, adding retention and drainage aids to the approach flow system, double-folding, laminating, pressing, drying, coating, calendering and reeling to obtain the high-performance environment-friendly kraft liner board.

7. The preparation method for the high-performance environment-friendly kraft liner board as recited in claim 6, wherein: the coating in the step (2) adopts a metering roller coating method, coating the flame retardant styrene-acrylic latex on the top layer of the kraft liner board obtained through double-folding, laminating, pressing and drying, so as to form a coating layer.

## Patentansprüche

1. Hochleistungsfähiger, umweltfreundlicher Kraftlinerkarton, umfassend eine untere Schicht, eine obere Schicht und eine Beschichtungsschicht, die nacheinander in einer Reihenfolge von unten nach oben angeordnet sind, wobei die untere Schicht aus einem Unterschicht-Zellstoff besteht, der aus einem modifizierten Holzpulver-Zellstoff und einem Kurzfaser-Zellstoff zusammengesetzt ist; wobei die obere Schicht aus einem Oberschicht-Zellstoff besteht, der aus einem Langfaser-Zellstoff und einem Kurzfaser-Zellstoff zusammengesetzt ist; wobei die Beschichtungsschicht durch Auftragen eines flammhemmenden Styrol-Acryl-Latex auf die obere Schicht gebildet wird; wobei der Langfaser-Zellstoff und der Kurzfaser-Zellstoff durch Zerkleinern alter Haushalts-Wellpappen gebildet werden; wobei der flammhemmende Styrol-Acryl-Latex aus modifizierten zusammengesetzten Flammschutzmitteln, einem funktionell modifizierten Styrol-Acryl-Latex und Wasser besteht; wobei die zusammengesetzten Flammschutzmittel eine Kombination aus zwei oder mehr von Ammoniumpolyphosphat, Polyphosphoester, Melaminpolyphosphat, Zinkborat, Aluminiumhydroxid und Aluminiumphosphat sind; wobei die modifizierten zusammengesetzten Flammschutzmittel durch Modifizierung von zusammengesetzten Flammschutzmitteln mit einem Silan-Kopplungsmittel hergestellt werden;
wobei das Gewichtsverhältnis der modifizierten zusammengesetzten Flammschutzmittel zu dem funktionell modifizierten Styrol-Acryllatex 1:2,5-3,0 beträgt; wobei die modifizierten zusammengesetzten Flammschutzmittel durch Modifizierung von zusammengesetzten Flammschutzmitteln mit einem Silan-Kopplungsmittel hergestellt werden; wobei der funktionell modifizierte Styrol-Acryl-Latex durch folgende Schritte hergestellt wird : Zugabe von Dicyclopentenylmethacrylat, Wasser, Natriumdodecylsulfat und Nonylphenolpolyoxyethylenether entsprechend einem Verhältnis in einen Reaktor 1, gleichmäßiges Rühren; Zugabe von Trimethylencarbonat, nach gleichmäßigem Rühren; sukzessive Zugabe von Acrylsäure, Hydroxyethylacrylat, Butylacrylat und Styrol in das Reaktionssystem, Rühren bei konstanter Geschwindigkeit, bis es gut vermischt ist; danach Erhitzen des Reaktionssystems auf 70-90° C, Zugabe von Natriumbicarbonat und einem Initiator, wobei unter Rühren eine Reaktion bei konstanter Temperatur für 2-4 Stunden durchgeführtwird, Abkühlen auf Raumtemperatur, Filtrieren, Einstellen des pH-Werts des erhaltenen Produkts auf neutral und Erhalten des funktionell modifizierten Styrol-Acryl-Latex, wobei der Anteil ein Gewichtsverhältnis des Dicyclopentenylmethacrylats, des Wassers, des Natriumdodecylsulfats, des Nonylphenolpolyoxyethylenethers, des Trimethylencarbonats, der Acrylsäure, des Hydroxyethylacrylats, des Butylacrylats, des Styrols, des Natriumbicarbonats und des Initiators von 1:40-50:0.2-0.3:0.3-0.4:1-1.3:0.2-0.5:4-6: 25-35:25-35:0.2-0.4:0.4-0.6, und wobei ein Grenzsauerstoffindex 30-33 % beträgt, eine Glätte 15-16 Sekunden beträgt, ein Berstindex 2,4-2,6 kPam²/g beträgt und eine Faltbeständigkeit 15-20-Fache beträgt.

2. Hochleistungsfähiger, umweltfreundlicher Kraftlinerkarton nach Anspruch 1, wobei das Flächengewicht des Hochleistungsfähigen, umweltfreundlichen Kraftlinerkartons 100 bis 120 g/m² beträgt, der Ringdruckindex 6,7-7,6 mNm²/g beträgt, die frontale Wasseraufnahme 30-31 g/m² beträgt.

3. Hochleistungsfähiger, umweltfreundlicher Kraftlinerkarton nach Anspruch 1, wobei das Dicyclopentenylmethacrylat durch folgende Schritte hergestellt wird:
nacheinander Zugabe von Methacrylsäure, Trifluormethansulfonsäure und Hydrochinon entsprechend einem Verhältnis in einen Reaktor 2, Rühren und gutes Mischen, Erhitzen auf 78-82°C, Zugabe von Dicyclopentadien in den Reaktor 2, gutes Mischen, dann Erhitzen des Reaktionssystems auf 85-90° C, wobei eine Reaktion bei konstanter Temperatur für 3-4 Stunden durchgeführt wird, Abkühlen auf Raumtemperatur nach Beendigung der Reaktion, Zugabe von Natriumhydroxid zum erhaltenen Produkt, Rühren für 12 Stunden, schließlich Waschen der erhaltenen Mischung, Filtrieren, Destillieren und Erhalten des Dicyclopentenylmethacrylats, wobei die Trifluormethansulfonsäure, das Hydrochinon, das Dicyclopentadien und das NaOH 0.8-1.2:0.002-0.004:0.00006-0.0001:1.5-2.0:0.0015-0.002.

4. Hochleistungsfähiger, umweltfreundlicher Kraftlinerkarton nach Anspruch 1, wobei ein Gewichtsverhältnis des Dicyclopentenylmethacrylats, des Wassers, des Natriumdodecylsulfats, des Nonylphenolpolyoxyethylenethers, des Trimethylencarbonats, der Acrylsäure, des Hydrox1:40-50:0,2-0,3:0,3-0,4:1-1,3:0,2-0,5:4-6:25-35: 25-35:0,2-0,4:0,4-0,6 ist.

5. Hochleistungsfähiger, umweltfreundlicher Kraftlinerkarton nach Anspruch 1, wobei der modifizierte Holzpulver-Zellstoff durch Modifizierung von Holzpulvern mit einem Quellmittel hergestellt wird und das Quellmittel ein Alkali-Gemisch ist; wobei ein Modifizierungsverfahren ist wie folgt: nach der Verarbeitung der Holzpulver mit einem Refiner werden nacheinander das gemischte Alkali und Wasser zugegeben, gleichmäßig gerührt, dann wird eine erhaltene Mischung auf 70-90°C erhitzt, und eine Quellungsbehandlung wird bei konstanter Temperatur für 60-90 Minuten durchgeführt, um den modifizierten Holzpulver-Zellstoff zu bilden; wobei das gemischte Alkali aus Natriumhydroxid und Natriumcarbonat besteht.

6. Herstellungsverfahren für einen Hochleistungsfähigen, umweltfreundlichen Kraftlinerkarton nach Anspruch 1, das die folgenden Schritte umfasst:
(1) Auflösungsschritte
(i) Herstellung eines Langfaser-Zellstoffs und eines Kurzfaser-Zellstoffs
Entflockung alter Haushalts-Wellpappen mit einem Hydrapulper, Abtrennung des Bodensatzes bei hoher Konsistenz, dann Grobsortierung auf der ersten Stufe in drei Stufen, Sortierung in einen Langfaser-Grobstoff und einen Kurzfaser-Grobstoff; Abtrennung des Langfaser-Grobstoffs auf der ersten Stufe in drei Stufen, Entfernung des Bodensatzes; sukzessive Feinsortierung der erhaltenen Fasern für die ersten drei Stufen, Sieben mit einem Mehrscheiben-Eindicker, Raffinieren mit einem konischen Refiner und abschließendes Verdünnen mit Wasser, um den Langfaser-Zellstoff zu erhalten, Lagerung in einer Maschinenkiste zur Verwendung;
anschließende Feinsortierung des Kurzfaser-Grobstoff für die ersten zwei Stufe und Mahlen mit dem konischen Refiner, schließlich Verdünnen mit Wasser, um den Kurzfaser-Zellstoff zu erhalten, Lagerung in einer Zellstoffkiste zur Verwendung;
(ii) Herstellung eines modifizierten Holzpulver-Zellstoffs
Verarbeitung von Holzpulvern mit einem Refiner, sukzessive Zugabe einer Alkalimischung und Wasser, gleichmäßiges Rühren, Erhitzen der erhaltenen Mischung auf 70-90°C, und Durchführung einer Quellbehandlung bei konstanter Temperatur für 60-90 Minuten, um die Fasern entsprechend zu erweichen und den modifizierten Holzpulver-Zellstoff mit einer Gewichtsprozentkonzentration von 3-5% zu bilden;
(2) Schritte der Papierherstellung
Mischen des modifizierten Holzpulvers und des in Schritt (1) erhaltenen Kurzfaser-Zellstoffs nach einem bestimmten Verhältnis, um einen Unterschicht-Zellstoff zu bilden,
gleichmäßiges Mischen des Langfaser-Zellstoffs und des Kurzfaser-Zellstoffs,
um einen Oberschicht-Zellstoff zu bilden;
Anschließend werden der Unterschicht-Zellstoff und der Oberschicht-Zellstoff jeweils auf ein Sieb geleitet, Retentions- und Entwässerungshilfen in das Konstantteilsystem eingebracht, doppelt gefaltet, laminiert, gepresst, getrocknet, gestrichen, kalandriert und aufgerollt, um den Hochleistungsfähigen, umweltfreundlichen Kraftlinerkarton zu erhalten.

7. Herstellungsverfahren für einen Hochleistungsfähigen, umweltfreundlichen Kraftlinerkarton nach Anspruch 6, wobei die Beschichtung in Schritt (2) ein Dosierwalzen-Beschichtungsverfahren anwendet, bei dem der flammhemmende Styrol-Acryl-Latex auf die obere Schicht des Kraftlinerkartons aufgetragen wird, die durch Doppelfalten, Laminieren, Pressen und Trocknen erhalten wird, um eine Beschichtungsschicht zu bilden.

## Revendications

1. Carton kraft doublé respectueux de environnement à haute-performance, comprenant une couche de fond, une couche de sommet et une couche de revêtement, qui sont disposées successivement dans un ordre de bas en haut; **caractérisé en ce que** ladite couche de fond est faite d'une pâte à papier de couche de fond composée d'une pâte modifiée à poudre de bois et d'une pâte à fibres courtes; ladite couche de sommet est faite d'une pâte à papier de couche de sommet composée d'une pâte à fibres courtes et d'une pâte à fibres longues; ladite couche de revêtement est formée par le moyen de revêtir un styrène-acrylique latex ignifuge sur ladite couche de sommet; la pâte à fibres courtes et la pâte à fibres longues sont formées par la mise en pâte de vieilles boîtes ondulées domestiques; le styrène-acrylique latex ignifuge se compose de retardateurs de flamme composés modifiés, un styrène-acrylique latex modifié fonctionnel et eau; les retardateurs de flamme composés sont une combinaison de deux ou plusieurs de un polyphosphate d'ammonium, un polyphosphoester, un polyphosphate de mélamine, un borate de zinc, un hydroxyde d'aluminium et un phosphate d'aluminium; les retardateurs de flamme composés modifiés sont préparés par le moyen de modifier les retardateurs de flamme composés avec un agent de couplage silane;
un rapport de poids entre les retardateurs de flamme composés modifiés et le styrène-acrylique latex modifié fonctionnel est 1:2,5-3,0; les retardateurs de flamme composés modifiés sont préparés par le moyen de modifier les retardateurs de flamme composés avec un agent de couplage silane;
le styrène-acrylique latex modifié fonctionnel est préparé par étapes de:
selon une proportion, ajouter du méthacrylate de dicyclopentényle, de l'eau, du dodécylsulfate de sodium et de l'éther polyoxyéthylène de nonylphénol dans un réacteur 1, en remuant uniformément; ajouter du carbonate de triméthylène, après l'avoir remué uniformément, ajouter successivement de l'acide acrylique, de l'acrylate d'hydroxyéthyle, de l'acrylate de butyle et du styrène dans un système de réaction, en remuant à vitesse constante jusqu'à bien mélanger; ensuite, chauffer le système de réaction à 70-90°C, et ajouter du bicarbonate de sodium et un initiateur de façon à faire une réaction à température constante pendant 2 à 4 heures dans des conditions d'agitation, à la fin de la réaction, refroidir le système à température ambiante, faire filtrage, ajuster de la valeur du pH d'un produit obtenu à neutre, puis obtenir le styrène-acrylique latex modifié fonctionnel, dans lesquelles la proportion inclut un rapport de poids du méthacrylate de dicyclopentényle, l'eau, le dodécylsulfate de sodium, l'éther polyoxyéthylène de nonylphénol, le carbonate de triméthylène, l'acide acrylique, l'acrylate d'hydroxyéthyle, l'acrylate de butyle, le styrène, le bicarbonate de sodium et le initiateur est 1 :40-50 :0.2-0.3 :0.3-0.4 :1-1.3 :0.2-0.5 :4-6 : 25-35 :25-35 :0.2-0.4 :0.4-0.6.

2. Carton kraft doublé respectueux de environnement à haute-performance selon la revendication 1, **caractérisé en ce que** du carton kraft doublé respectueux de environnement à haute-performance, un grammage est 6.7-7.6 mN·m²/g, une absorption de l'eau frontale est 30-31 g/m², un indice limite d'oxygène est 30-33%, une planitude est 15-16 secondes, un indice de pétardage est 2.4-2.6 kPa·m²/g, une endurance de pliage est 15-20 fois.

3. Carton kraft doublé respectueux de environnement à haute-performance selon la revendication 1, **caractérisé en ce que** le méthacrylate de dicyclopentényle est préparé par étapes de :
selon une proportion, ajouter successivement de l'acide méthacrylique, de l'acide trifluorométhanesulfonique et de l'hydroquinone dans un réacteur 2, après les avoir remués et mélangés, les chauffer à 78-82 °C, ajouter du dicyclopentadiène au réacteur 2, en les ayant mélangés, puis chauffer le système de réaction à 85-90 °C de façon à faire une réaction à température constante pendant 3 à 4 heures, à la fin de la réaction, refroidir le système à température ambiante, ajouter de l'hydroxyde de sodium dans un produit obtenu, en les remuant pendant 1 à 2 heures, puis laver un mélange obtenu, filtrer et distiller le mélange, enfin obtenir le méthacrylate de dicyclopentényle, dans lesquelles la proportion inclut un rapport de poids de l'acide trifluorométhanesulfonique, l'hydroquinone, le dicyclopentadiène et le NaOH est 0.8-1.2:0.002-0.004:0.00006-0.0001: 1.5-2.0:0.0015-0.002.

4. Carton kraft doublé respectueux de environnement à haute-performance selon la revendication 1, **caractérisé en ce que** la proportion inclut un rapport de poids du méthacrylate de dicyclopentényle, l'eau, le dodécylsulfate de sodium, l'éther polyoxyéthylène de nonylphénol, le carbonate de triméthylène, l'acide acrylique, l'acrylate d'hydroxyéthyle, l'acrylate de butyle, le styrène, le bicarbonate de sodium et le initiateur est 1:40-50:0.2-0.3:0.3-0.4:1-1.3:0.2-0.5:4-6:25-35:25-35:0.2- 0.4:0.4-0.6.

5. Carton kraft doublé respectueux de environnement à haute-performance selon la revendication 1, **caractérisé en ce que** la pâte modifiée à poudre de bois est préparée par le moyen de modifier les poudres de bois avec un agent gonflant, le agent gonflant est un alcali mixte; une méthode de modification est effectuée par étapes de : après avoir traité les poudres de bois avec un raffineur, ajouter successivement l'alcali mixte et l'eau, en les remuant uniformément, puis chauffer un mélange obtenu à 70-90°C de façon à faire un traitement de gonflement à température constante pendant 60 à 90 minutes, enfin former la pâte modifiée à poudre de bois, dans lesquelles l'alcali mixte se compose d'hydroxyde de sodium et carbonate de sodium.

6. Méthode de préparation pour le carton kraft doublé respectueux de environnement à haute-performance selon la revendication 1, comprenant les étapes de:
(1) dans une étape de mise en pâte
(i) préparer une pâte à fibres courtes et une pâte à fibres longues,
- casser vieilles boîtes ondulées domestiques à l'aide d'un hydrapulpeur, séparer des déchets à haute consistance, puis les cribler grossièrement pour premières trois étapes, en les criblant à une pâte grossière à fibres courtes et une pâte grossière à fibres longues, -séparer la pâte grossière à fibres longues pour premières trois étapes, et éliminer des déchets;
- cribler finement des fibres obtenues pour premières trois étapes successivement, en les épaississant à l'aide d'un épaississeur multidisques, et les raffinant à l'aide d'un raffineur conique, enfin les diluant avec de l'eau pour obtenir la pâte à fibres longues, puis la mettre en réserv dans un calow;
- cribler finement la pâte grossière à fibres courtes pour premières deux étapes successivement, en la raffinant à l'aide du raffineur conique, enfin la diluant avec de l'eau pour obtenir la pâte à fibres courtes, puis la mettre en réserv dans un calow;
(ii) préparer une pâte modifiée à poudre de bois,
- traiter des poudres de bois avec un raffineur, ajouter du alcali mixte et de la eau successivement, en les remuant uniformément, pius chauffer un mélange obtenu à 70-90°C de façon à faire un traitement de gonflement à température constante pendant 60 à 90 minutes, afin d'assouplir les fibres de manière appropriée et de former la pâte modifiée à poudre de bois avec une concentration en pourcentage de poids de 3 à 5%;
(2) dans une étapes de fabrication du papier
- selon une proportion, mélanger uniformément la pâte modifiée à poudre de bois et la pâte à fibres courtes obtenues par l'étape (1) pour former une pâte à papier de couche de fond,
- mélanger uniformément la pâte à fibres longues et la pâte à fibres courtes pour former une pâte à papier de couche de sommet;
- puis laisser couler la pâte à papier de couche de fond et la pâte à papier de couche de sommet sur un filet de papeterie respectivement, additionner des équipements auxiliaires de rétention et drainage au système d'empesage, faire double pliage, laminage, pressage, séchage, enduction, calandrage et enroulage pour obtenir le carton kraft doublé respectueux de environnement à haute-performance.

7. Méthode de préparation selon la revendication 6, **caractérisé en ce que** la enduction de l'étape (2) adopte une méthode de enduction à rouleau doseur, revêtant le styrène-acrylique latex ignifuge sur ladite couche de sommet du carton kraft doublé obtenue par double pliage, laminage, pressage et séchage, de manière à former une couche de revêtement.
